

(No Model.)

M. H. KNAPP.

CRUCIBLE.

No. 251,719.

Patented Jan. 3, 1882.

Fig. 1



Fig. 2



Attest:

A. Barthel  
E. Scully.

Inventor:

Milton H. Knapp  
per Thos. Spague  
Attr.

# UNITED STATES PATENT OFFICE.

MILTON. H. KNAPP, OF ADRIAN, MICHIGAN.

## CRUCIBLE.

SPECIFICATION forming part of Letters Patent No. 251,719, dated January 3, 1882.

Application filed September 28, 1881. (No model.)

*To all whom it may concern:*

Be it known that I, MILTON H. KNAPP, of Adrian, in the county of Lenawee and State of Michigan, have invented an Improvement 5 in Crucibles, of which the following is a specification.

The nature of this invention relates to certain new and useful improvements in the manufacture of crucibles especially designed for 10 dentists' and jewelers' use in melting metals, although I intend not to confine myself to the small crucibles used in those professions, but make them of any size required. In such crucibles the metal is usually melted under the 15 action of heat directed and accelerated by the blast of a blow-pipe, and this strong blast, intensifying the heat as it does, has a tendency rapidly to destroy and render entirely useless the best crucibles now to be found in the market.

20 The object of my invention, therefore, is to provide a crucible which will not be injured or destroyed under those circumstances.

Figure 1 represents a crucible for dental purposes unattached. Fig. 2 represents the same 25 in a ladle or metallic crucible with a handle, by which to support it.

In the accompanying drawings, which form a part of this specification, A represents a crucible for dentists' use, in which to melt metals 30 employed for dental purposes. The main feature of this crucible is in the employment of asbestos in its construction. This may be done

by the use of what is known as "mill-board," which is made of asbestos fiber mixed with a little paper-stock. When made of this board 35 the heat to which it is subjected in use will destroy the paper-stock, and then, if undue pressure is brought to bear upon the crucible, it will break down unless supported in a ladle or other suitable device, as shown in Fig. 2. 40

I do not desire to confine myself to the use of mill-board, for the asbestos fiber may be pressed into the required shape under proper pressure and in suitable dies, and in such case the crucible thus formed would be necessary 45 to be sustained by being placed within a metal crucible or ladle.

I am aware that it is not new to protect crucibles with an outer coating or shield of asbestos, and therefore I do not claim such invention. 50

What I claim as my invention is—

1. A crucible composed of asbestos fiber and paper-stock mixed and molded into shape, substantially as described.

2. A crucible made in two parts, the inner 55 one composed of asbestos fiber and paper-stock mixed and pressed into shape and the outer part made of metal for supporting the inner part, substantially as described.

MILTON H. KNAPP.

Witnesses:

C. A. STACY,  
A. L. MILLARD.